

E. E. ALLYNE.

PISTON.

APPLICATION FILED JAN. 9, 1919.

1,426,138.

Patented Aug. 15, 1922.



Inventor

Edmund E. Allyne

By

Ray A. Gehr

Attorney

# UNITED STATES PATENT OFFICE.

EDMUND E. ALLYNE, OF CLEVELAND, OHIO, ASSIGNOR, BY MESNE ASSIGNMENTS, TO  
ALUMINUM MANUFACTURES, INCORPORATED, OF CLEVELAND, OHIO, A CORPO-  
RATION OF DELAWARE.

## PISTON.

1,426,138.

Specification of Letters Patent. Patented Aug. 15, 1922.

Application filed January 9, 1919. Serial No. 270,318.

To all whom it may concern:

Be it known that I, EDMUND E. ALLYNE, a citizen of the United States, residing at Cleveland, in the county of Cuyahoga and 5 State of Ohio, have invented certain new and useful Improvements in Pistons, of which the following is a specification, reference being had therein to the accompanying drawings.

10 This invention relates to improvements in pistons for internal combustion engines and to the process of producing said pistons. It relates especially to pistons made of aluminum alloys or other light weight 15 metals which are subject in operation to corrosion resulting in so called "pitting".

The principal object of the invention is the production of pistons of materials of 20 the character referred to which will be substantially unaffected by those operating conditions which cause pitting of pistons of such materials heretofore used.

To this end I provide the piston made of 25 aluminum alloy, or other material subject to pitting, with a protective layer or coating of material, preferably metal, which is not subject to corrosion under the conditions of operation. The pitting action is usually localized, affecting only certain 30 parts of the top or side piston surfaces which are exposed to the gases of the combustion chamber, and in the practice of my invention it is necessary to provide the protective coating only for those parts 35 which are found to be subject to the pitting action.

In order that my invention may be clearly understood I will describe in detail its application to pistons of aluminum alloy.

40 In the carrying out of my improved method of making pistons the first step is the production of an aluminum alloy piston of the desired form and construction in any known manner, for example, by casting, machining and finishing.

The next step is to determine whether 45 such piston will be subject to corrosion in the particular engine in which it is to be used, and if so, where the corrosion will occur. As has been indicated above, the pitting action is more or less definitely localized. Several theories have been advanced

in explanation of the action. The main casual factors involved seem to be a relatively high temperature inducing either 55 chemical corrosive action, such as oxidation, on the metal of the piston by the combustion gases or a softening or melting of the metal, and the mechanical action of localized currents of the combustion gases as they enter 60 or leave the cylinder or during combustion.

Whatever the true explanation may be, it is difficult to predict whether or not the pistons of a particular engine will be subject to pitting and where the pitting will 65 appear, if it does occur. In some cases the location of the pitting seems to bear a certain relation to the spark plug or the intake passage, or both. In other cases no such definite casual relation can be perceived. The only satisfactory and sure 70 way to determine this is to make an actual trial of the engine under the most severe operating conditions. If pitting occurs, its location is thus determined and my improved protective coating can then be applied to the pistons to be used in the same 75 and similar engines so as to cover and protect the area or areas where pitting would occur.

The location of the pitting having been determined, in one way or another, the next 80 step of my improved process is the application of the protective coating. In the production of aluminum alloy pistons several different protective coatings have been 85 employed with more or less complete success. The most satisfactory results have been secured with iron, nickel and copper. Any one of these metals can be used or any 90 two or more of such metals. For example, a coating may consist of iron covered with copper, or iron covered with nickel, or of other various combinations of these or other suitable metals. As I am at present advised, the best results are obtained from a coating composed of a layer of iron upon 95 which is superposed a layer of nickel.

The coating may be of any thickness suitable to insure protection of the underlying 100 metal subject to corrosion and may be applied in any suitable manner. Obviously where light weight is a desideratum the coating should not be any thicker than

necessary to afford the desired protection. In many cases a coating of iron or iron and nickel from one thousandth to two thousandths of an inch in thickness is found to 5 afford adequate protection.

While, as stated above, the protective coating may be applied to the piston in any suitable manner, the fact that only a portion of the piston surface need be treated, 10 as well as other considerations, make the electrolytic depositions of the coating especially advantageous. In applying the coating by this method the area to be covered is first cleaned and polished and otherwise treated as may be necessary for the 15 reception of a firm and adherent coating of the material. The piston is then placed in the plating tank and the metal or metals deposited thereon in a well known manner. 20 The piston is then removed from the plating bath and all deposited metal removed except that which covers the area to be protected. The removal of this extra metal is easy because it does not adhere well to aluminum alloy surfaces which have not been 25 especially treated or prepared and it may, therefore, be easily brushed off. The piston is then ready for use. In cleaning the piston surfaces as above described, any suitable known material and procedure can be 30 employed, and any suitable known electrolyte can be used.

In order that the invention may be quite clearly understood I have illustrated in the 35 accompanying drawings a piston constructed in accordance with my invention to obviate the pitting which has been found to occur in one type of engine.

In the drawings, 40 Figs. 1 and 2 are a side elevation and plan, respectively, of a piston embodying my improvements.

Fig. 3 is a transverse vertical section through the upper part of a cylinder of an 45 internal combustion engine with one of my improved pistons shown in elevation.

Fig. 4 is a horizontal section on the line 4-4, Fig. 3.

Fig. 5 is a vertical section on the line 50 5-5, Fig. 3.

The piston illustrated in Figs. 1 and 2 is of the type used in the Liberty aviation motor. It is cast from aluminum alloy and comprises a head section 1 having a top 55 surface 1<sup>a</sup> and a side surface 1<sup>b</sup>, a skirt 2, and pin bosses 3, 3. 4, 4 are the usual packing rings.

The piston has a portion of its top wall 1<sup>a</sup> and of its side wall 1<sup>b</sup> provided with a 60 protective coating 5, preferably of iron and nickel electrolytically deposited as herein above described.

In Fig. 3 the piston is shown mounted in the engine cylinder 6. The cylinder is provided with an intake passage 7, an exhaust

passage 8 and a spark plug 9. In this particular type of engine it was found that pitting of the aluminum alloy pistons occurred in a region adjacent the intake passage and the spark plug and it will be observed that the protective coating covers this part of the piston. 70

While it seems probable that the pitting of aluminum alloy pistons is due to oxidation or other corrosive chemical action by 75 the combustion gases, some who have studied the matter incline to the view that the pitting results from a melting of the alloy, or at least of the eutectic portion of the alloy, due to exceedingly high temperatures 80 in the combustion chamber, such melting or softening of the metal being followed by the erosive or disintegrating action of the gas currents on the softened metal. In this connection it will be observed that the coating metals which I have herein above specified for use on aluminum alloy pistons, have considerably higher melting points than does the aluminum alloy so that my 85 invention provides an effective remedy for 90 pitting whether it results from chemical action or an actual melting of the metal, or from both of these actions.

It is to be noted that whereas certain of 95 the various specified coating metals may not be entirely resistant to corrosion when they alone comprise a complete piston, they are all rendered noncorrodible when intimately attached to an aluminum alloy piston as 100 herein disclosed. Although the true reason for this result is not definitely known to me, I believe it to be due to the maintenance of the coating metal at a comparatively 105 low temperature. Aluminum and its alloys absorb and conduct heat more rapidly than many metals, such for example as iron. Accordingly an aluminum alloy piston will absorb heat from the coating metal and rapidly conduct it away to other parts of the piston, thus maintaining the coating metal 110 at a relatively low temperature at which it is not corrodible by the gases in the engine.

It is obvious that the relatively thin protective coating such as I have described does not add materially to the weight of the piston so that light weight alloy pistons constructed in accordance with my invention possess all of the desired properties of pistons of this character and are at the same time free from the harmful pitting action 115 to which such pistons are subject.

It will be understood that while the invention is especially useful in connection with pistons of aluminum alloy or the like, in its broader aspects it is not limited to 120 such materials but is applicable to any piston material subject to corrosive pitting to which a non-corrodible protective coating can be applied. It will also be understood 125 that the method of applying the protective 130

coating can be widely varied and that the foregoing description and the accompanying drawings have been set forth for purpose of explanation and illustration and are not intended to define the scope of the invention.

What I claim is:

1. A piston for internal combustion engines composed of aluminum alloy and having on that part exposed to the combustion gases means for protecting the aluminum alloy from the corrosive action of said gases, said means comprising a coating of

iron intimately united to the aluminum alloy.

2. A piston for internal combustion engines composed of aluminum alloy and having on that part exposed to the combustion gases means for protecting the aluminum alloy from the corrosive action of said gases, said means comprising a coating of electrolytically deposited iron intimately united to the aluminum alloy of the piston.

In testimony whereof I hereunto affix my signature.

EDMUND E. ALLYNE.